

## UNITED STATES PATENT OFFICE

2,293,237

## HYDROCARBON PRODUCT

Jeffrey H. Bartlett, Cranford, N. J., assignor to  
Standard Oil Development Company, a corpora-  
tion of Delaware

No Drawing. Application December 29, 1939,  
Serial No. 311,523

6 Claims. (Cl. 252—47)

The present invention relates to an improvement in lubricants and similar oils, as well as other hydrocarbon materials, especially in respect to resistance to decomposition at elevated temperatures under oxidizing conditions such as are encountered in internal combustion engines. The invention will be fully understood from the description which follows.

It has been found that mineral oil lubricants can be greatly improved in respect to their stability against decomposition, especially under heat and oxidizing conditions, by addition thereto of small amounts of certain substances. In the present case, a new group of substances has been discovered which are particularly effective in reducing the oxidation of oils at elevated temperatures. This group of substances comprises the peri-naphthothiazines and their derivatives, which may be defined by the formula



in which R, R', and R'' may be hydrogen, halogen, amino, mercapto, hydroxyl, or an organic group, such as alkyl, aryl, alkoxy, aroxy, -NH-alkyl, -NH-aryl, -N-alkyl, -N-aryl, -S-alkyl, -S-aryl, or an organic group containing a heterocyclic ring structure. There may be more than one such substituent group attached to either or both of the carbon rings.

The following are examples of this class of compounds:



2-methyl-peri-naphtho-m-thiazine



2-(m-hydroxyphenyl)-peri-naphtho-m-thiazine

The new class of antioxidant compounds are advantageously added to the oils in concentra-

tions ranging from about 0.01% to about 1%, but the quantity generally preferred is about 0.1%.

The addition agents of this invention do not have any detrimental effects on the physical character of the lubricating oil or the mineral oil to which they are added, such as viscosity, gravity and flash point. The present materials may be used as the sole blending agents, or they may be added, in the case of a lubricant, with other ingredients which serve other purposes. They are useful agents to be added to leaded oils, that is to say, lubricants containing lead oleate, lead naphthenate, lead sulfonate or other heavy metal soaps. They also may be added along with oiliness agents, pour depressants, lubricating oil dyes, or agents to give fluorescence. They may be used in conjunction with any other antioxidants or with thickeners, sludge or sediment dispersers and the like.

The value of the antioxidants of the present invention when used in lubricating oil blends has been determined by a standard oxygen absorption test. This test is used for the most part in judging the oxidation susceptibility of a lubricating oil at engine operation temperatures. A known amount of oxygen is bubbled through 10 cc. of the lubricating oil maintained at 200° C. The oxygen is continuously recycled. At the end of successive 15 minute periods, the amount of oxygen absorbed by the oil is measured. The results, usually termed the oxidation rate of the oil, are given as the number of cubic centimeters of oxygen absorbed by 10 cc. of an oil per 15 minute intervals at 200° C.

The following examples illustrate the value of the new class of antioxidants in accordance with the present invention.

*Example 1*

A refined mineral lubricating oil having a viscosity of 87 seconds (Saybolt) at 210° F. and containing no antioxidant was tested for its oxygen absorption rate according to the standard test described above. The number of cubic centimeters of oxygen absorbed in three successive 15 minute intervals were 103, 213 and 107, respectively.

*Example 2*

A blend of the base oil described in Example 1 with 0.1% of 2-methyl-peri-naphtho-m-thiazine, a yellow crystalline compound, which may be prepared according to the method described in Jour. Amer. Chem. Soc., 53:4050 (1931), was tested for its oxidation rate as above, and the rates for three successive 15 minute intervals were found to be 15, 24 and 31, respectively.

*Example 3*

A blend of the base oil described in Example 1

with approximately 0.2% of 2-(m-hydroxy-phenyl)-peri-naphtho-m-thiazine, an orange crystalline compound, which may be prepared according to the method described in Jour. Amer. Chem. Soc., 53:4056 (1931), was tested for its absorption rate in the manner described, and the rates for four successive 15 minute intervals were 14, 14, 18 and 20, respectively.

The present invention is not to be considered as limited by any of the herein described examples, which are given by way of illustration only, but is to be limited solely by the terms of the following claims in which it is desired to claim all novelty inherent in the invention.

I claim:

1. An improved lubricant comprising a mineral lubricating oil and a small quantity of a compound of the formula:



in which R, R' and R'' are selected from the class consisting of hydrogen and halogen atoms and amino, mercapto, hydroxyl and organic groups.

2. An improved lubricant comprising a mineral lubricating oil and a small quantity of 2-methyl-  
peri-naphtho-m-thiazine.
3. An improved lubricant comprising a mineral lubricating oil and about 0.1% of 2-methyl-  
peri-naphtho-m-thiazine.
4. An improved lubricant for use at elevated temperatures comprising a lubricating oil and about 0.01% to about 1.0% of a compound of  
10 the formula:



in which R, R' and R'' are selected from the class consisting of hydrogen and halogen atoms and amino, mercapto, hydroxyl and organic groups.

5. An improved lubricant comprising a mineral lubricating oil and a small quantity of 2-(m-hydroxyphenyl)-peri-naphtho-m-thiazine.

6. An improved lubricant comprising a mineral lubricating oil and about 0.2% of 2-(m-hydroxyphenyl)-peri-naphtho-m-thiazine.

JEFFREY H. BARTLETT.